

July 3, 1923.

1,460,703

J. G. CAPSTAFF

PHOTOGRAPHIC REVERSAL PROCESS

Filed March 1921

FIG. 1.



FIG. 2.

WITNESS

*James H. Stewart.*

INVENTOR

John G. Capstaff,  
BY P. L. Strinchfield  
H. M. Penning  
ATTORNEYS.

## UNITED STATES PATENT OFFICE.

JOHN G. CAPSTAFF, OF ROCHESTER, NEW YORK, ASSIGNOR TO EASTMAN KODAK COMPANY, OF ROCHESTER, NEW YORK, A CORPORATION OF NEW YORK.

## PHOTOGRAPHIC REVERSAL PROCESS.

Application filed March 2, 1921. Serial No. 449,249.

*To all whom it may concern:*

Be it known that I, JOHN G. CAPSTAFF, a citizen of the United States of America, residing at Rochester, in the county of Monroe and State of New York, have invented certain new and useful Improvements in Photographic Reversal Processes, of which the following is a full, clear, and exact specification.

10 My invention relates to the making of positive pictures upon the same support and in the same sensitive layer that is exposed in the camera, and more particularly is an improvement in the method known as 15 "reversal," in which a negative silver image is made by exposure and development, this silver image being removed from the undeveloped silver salts, which are then converted into a positive image.

20 One of the great obstacles to the successful practice of this method is the necessity for such exact exposure and development that there will be left, after the removal of the developed negative silver image, an image 25 in the undeveloped salt that reproduces correctly the tones of the original subject. As it is generally expressed, there is no latitude in the exposure. Moreover, any slight inequalities in the emulsion or variations of 30 the emulsion as a whole from the standard produce objectionably non-uniform positives.

I have perfected a process by which it is possible to allow as great latitude in the 35 original exposure as is permissible in making exposures for the production of negatives to be used in the customary printing methods. I would mention as pre-eminently important the controlled exposure to light of 40 the sensitive silver salts remaining after the removal of the developed negative silver image, in a step analogous to the printing of a positive from a negative. This will be more fully described hereinafter, with many 45 other new steps and refinements in the process contributing to the result mentioned and making possible the production of positives of uniform quality, all of which I consider parts of my invention, as more precisely defined in the claims.

In order to make the process clear, I will first outline very briefly the important steps so that the relations of each step and the details thereof to the whole process may not be obscured. I will then describe fully and

precisely the exact formulæ and materials used in my preferred process and indicate what precautions and care are necessary, and to what extent the steps may be varied and equivalents introduced. Following this, I will make some general remarks pertinent to the process as a whole.

While this process is of general application, it has been developed particularly with a view to use in the making of motion picture positives upon the film exposed in the camera, and I will describe the preferred process as applied to a strip of motion picture film embodying a long band consisting of a support of a cellulose ester composition coated with a silver bromide gelatine emulsion.

It is to be understood that the process as completely given below is illustrative and that I do not limit myself to the details thereof. These are given with a considerable degree of particularity in order that others may know fully the methods which I preferably follow. Other equivalent steps and formulæ may be used, and the features of novelty which I describe and claim may be introduced into processes differing considerably from those here given.

Referring to the accompanying drawing: Fig. 1 illustrates schematically the means used for determining the characteristics of the film, and

Fig. 2 illustrates the arrangement of the room in which the printing is done.

The steps of the complete preferred process are as follows:

1. Expose in the camera.
  2. Develop, resulting in a silver negative image in a sensitized layer.
  3. Wash.
  4. Reverse, i. e., remove the silver image.
  5. Wash.
  6. Clear in a bisulfite bath, removing products formed in step 4.
  7. Rinse.
  8. Ascertain characteristics of the film.
  9. Bathe in an alkali bath.
  10. Rinse.
  11. Expose to a controlled printing light.
  12. Develop.
  13. Rinse.
  14. Fix in an "acid-hypo" bath, removing undeveloped silver salts.
  15. Wash and dry.
- I will now describe the steps fully.

1. The exposure is made in the camera in the usual way. In all photographic processes there is a certain permissible variation in exposure consistent with the obtaining of the best results, and a further variation permitting passable or printable results. In reversal processes this latitude of exposure is extremely small and exposures must be very exact to obtain at all satisfactory results. In ordinary photographic processes, particularly with the materials and processes such as are used in ordinary hand camera work, this latitude is very great. While it is desirable with my process as with any other photographic process that this exposure be carefully timed, it is possible to vary it in substantially the same degree as in ordinary amateur hand camera work. The exposure, moreover, is made directly on the emulsion surface and not through the support as is necessary in many reversal processes.

2. The developer used should be a "contrasty" one, by which I mean one producing in the silver negative image a high degree of contrast or high "gamma" as it is denoted in photographic literature; and the development should be continued until all exposed grains have been developed, or to "gamma infinity" as it is denoted in photographic literature. If only partial development is given, the contrasts will be incorrectly rendered.

I first take the following developer:

35 A.

|                   |          |
|-------------------|----------|
| Sodium bisulphite | 25 gms.  |
| Hydroquinone      | 25 gms.  |
| Potassium bromide | 25 gms.  |
| 40 Water to       | 1 liter. |

B.

|                  |          |
|------------------|----------|
| Sodium hydroxide | 50 gms.  |
| Water to         | 1 liter. |

45 this being a known "process" developer. The following formulæ is then made up.

|                                   |             |
|-----------------------------------|-------------|
| A+B, equal parts                  | 3 liters.   |
| Sodium thiosulfate (30% solution) | 25 c. c.    |
| Formalin                          | 10-30 c. c. |

The film is developed in this for five minutes at 65° F.

55 The sodium thiosulfate and formalin are not indispensable; but, particularly with fast emulsions, the former gives improved results in that the high lights are clearer than are otherwise obtainable, and the formalin 60 acts as a hardener and is desirable to prevent reticulation of the gelatin in the later steps, particularly the alkali bath. The formula given is merely a typical one, a very great deal of variation being permissible in 65 it, consistent with satisfactory results.

3. This washing should remove all soluble halides, since as will be pointed out these tend to precipitate developable silver salts in the high-lights of the picture in the reversing bath. I find that washing for 5 to 70 10 minutes in running water is necessary and sufficient.

4. The film is now submitted to a reversing bath, preferably the following:

|                                      |           |
|--------------------------------------|-----------|
| Potassium permanganate (4% solution) | 1 part.   |
| Sulphuric acid (20%)                 | 1 part.   |
| Water                                | 20 parts. |

It is understood that if a long strip of motion picture film is being treated it will be wound on a drum or reel prior to development and kept thereon through all the steps. During this reversing process this reel is rapidly rotated, or the sensitive element is kept in vigorous motion by other means, as otherwise a heavy deposit, presumably of manganese dioxide, collects in the form of a metallic lustre on the surface of the film and has a strong tanning effect on the gelatine which retards the dissolving of the negative image. The "bleaching" or "reversing" is continued until the silver has been entirely dissolved or removed from the sensitive layer, leaving only the unexposed and undeveloped silver salts. Other oxidizing baths such as acid bichromate or any bath that dissolves out the silver leaving the silver halide salts, may be used. These baths should not, however, contain any soluble salts capable of forming insoluble silver compounds, as by reaction with the silver sulphate, as these would prove objectionable in the later steps of the process. The undeveloped salts are rendered insensitive by the presence of the oxidizing bath and by manganese dioxide or other products; and any latent image on the salts is destroyed so that the element may be exposed to white light before and during this bath without damage.

5. The element is then washed.

6. It is then submitted to a clearing bath of sodium or potassium bisulfite or to any other bath capable of removing from the film the manganese compounds or any other products that may have been formed in the bleaching operation. I customarily use a 1 to 2% aqueous solution of sodium bisulfite to which I submit the sensitive element for about five minutes. This restores to the undeveloped silver salts, at least in part, their sensitiveness which had been lost by the presence of the manganese dioxide or other products of the "bleaching" or "reversing" bath. It is desirable for uniform results that a standard bath at standard temperature be used. I have at this step a sensitive emulsion from which the silver image has been removed. On examination this appears as a more or less translucent layer in which

is a transparent image, the greatest transparency being where the greatest amount of silver was removed, that is, in the high lights of the original subject; and the image is there positive. It is, naturally, inert since it is substantially of gelatine only. Of course, there will not as a rule be a completely transparent image extending completely through the emulsion but there will be an inert and transparent image located within the undeveloped silver salts in the emulsion.

7. The element is then rinsed.

8. I next ascertain the characteristics of the film. It has been customary hitherto in reversal processes to expose the undeveloped sensitive salts to the action of light, frequently bright sunlight, whereby all particles were rendered developable, the only control being in the development, or by reduction or intensification, all of which are unsatisfactory as methods of compensating for non-uniform original exposures. I have discovered that the sensitive layer containing the unaffected sensitive salts from which have been removed the developed silver particles is differentially sensitive in such a way that it may be treated like a uniform emulsion of sensitive material upon which is a negative image, and when exposed to a printing light a developable image is made in the sensitive layer, the density of which may be controlled by the intensity and duration of the printing light. If the original picture was given a full exposure the amount of silver developed will be large and the amount of the silver salt removed will be correspondingly great. I find that the greater the first exposure and the more silver developed and removed, the less sensitive is the remaining silver salt, so that such a film requires a greater exposure for printing than one in which considerable salt was left following a light exposure. The exposure required in printing may be roughly judged by the eye but preferably is measured by some means. In treating a strip of motion picture film, I cut off at this stage a strip containing a series of picture areas, and expose them for a standard time to a standard light beneath a series of different known density areas. Any other means of testing by means of varied standardized light may be used. The resulting prints when developed will vary in density. A schematic showing of such an arrangement is to be found in Fig. 1, wherein F indicates a strip of motion picture film which has been carried through the steps 1 to 7, heretofore described. The strip W has a series of areas A of successively different density. These are exposed to a printing light L in a suitable lamp box B, having a light diffusing screen S and a transparent window P. While the window, film, and density strip are here indicated as separated,

this is done for purposes of clear illustration to show their relative positions, and it is to be understood that in use they would be in contact. I select the one which I consider best and from a known relation between this and my printing light determine the printing period for the reel of film. This trial print also enables me to determine the contrast of the film, and to prepare a suitable developing bath.

This test gives me information concerning another characteristic of the film. It sometimes happens, particularly when the original film was underexposed that a second reversal will take place at the second development. The test film indicates such a possibility. The test, therefore, gives me information as to three characteristics of the film, its printing value, its contrast and its liability to re-reverse; which three characteristics affect its future treatment respectively in printing, developing and the alkali bath.

9. If the tendency to re-reverse is not present, as is usually the case, this step is omitted. If, however, it is present, the film is submitted to an alkali bath, customarily a 0.1% aqueous solution of potassium hydroxide. Other alkaline baths may be used. There is a tendency in warm weather for the gelatine to reticulate in the alkali bath, even though it has been hardened, particularly if the bath is prolonged to seven minutes or over, or if it is at all warm. I, therefore, submit the element to the alkaline bath for three minutes at a temperature of not over 65° F.

This step may be of value in reversal processes, differing in detail from that here described. The tendency to re-reverse I have noted particularly when the original exposure was less than it should have been; and even then it usually seemed to be a result of faulty manipulation in the later photographic steps. When all the steps are properly carried out it does not seem to be present. The step is, nevertheless, a generally useful one, since errors in manipulation are not always easily avoided. This step, it will be noted, is of particular use in connection with the controlled exposure, step 11, since the tendency to re-reverse is not present in those reversal processes where this exposure is not controlled and all the remaining salts are exposed and developed. This step may be given, of course, where no test is made; and it may be given, if desired, as a regular procedure, either before or after the test is made.

After submission to the alkaline bath a sample may be again tested.

10. The element is then rinsed.

11. The film is now exposed by revolving the reel in a room lighted by diffused light from a standard source at a standard distance

70

75

80

85

90

95

100

105

110

115

120

125

130

from the reel. A sketch of such a room R is shown in Fig. 2, the film F being wound on a reel or drum D, supported by trunnions T resting in seats L in the standards M, and having a handle H by which it may be rotated. The lamps E are in the box Q with a diffusing from G, and are controlled with an electric switch I, by which current from a suitable source, not indicated, is applied to the wires K. Any suitable chronometer C may be used by the operator for timing the exposure. A dark room lamp N with a screen O transmitting non-actinic rays is also shown. The duration of the exposure to the standard light is determined by the test already described. I use a light that will print average exposures satisfactorily in about a minute, permitting the reel to be revolved many times and giving uniform exposure throughout its length. The standardizing of any particular measuring means with the printing light used is, of course, to be determined by the operator by trial with the lighting conditions of his workroom. The exposure may be made of constant duration and the light intensity varied as by the rheostat X.

If the film should get accidentally over-exposed or light struck at this time it can be de-sensitized and resensitized before redevelopment by resubmission to the reversing bath (step 4) and the clearing bath, (step 6), and again printed.

12. The sensitive element is now developed in safe light in any desired developer, and I find that a very wide range of developers may be used with satisfactory results. Having determined the contrast in the test strip already taken, it is possible that by appropriate choice and use of developer to modify the contrast of the finished pictures. For general use I find the following typical developer satisfactory:

|                                       |            |
|---------------------------------------|------------|
| 45. Monomethyl paramidophenol sulfate | 23 gms.    |
| Sodium sulphite                       | 500 gms.   |
| Hydroquinone                          | 92 gms.    |
| Sodium carbonate                      | 50 gms.    |
| Potassium bromide                     | 10 gms.    |
| 50. Water                             | 10 liters. |

While I preferably use a developer of the type generally known as "M-Q", I find that the proportion in this may be varied within wide limits and that practically any of the well known and standard developing agents and formulæ may be used at this stage. By varying the agents, proportions, dilutions, and temperature the contrast of the resulting image may be controlled in a manner that is known to any practical photographer.

In reversal processes such as I have already referred to in which the exposure to light is coincident with the redevelopment, the exposure may be controlled in similar

manner, but it is much more difficult to insure uniform printing in this way. In this case the reel D is mounted in the lower seats B, so that as it is rotated the lower portion will pass through the developing tank or tray Y.

13. The sensitive element is then rinsed.

14. It is then submitted to the usual acid thiosulfate fixing bath which dissolves out all the remaining undeveloped sensitive salts, after which it is washed and dried as usual. These steps may be performed in ordinary light.

While it is simplest to perform all the steps in succession on the film or other sensitive element, without drying between the steps, it is possible to perform the steps at different times, drying the element between the steps. While I have described the use of motion picture film more particularly it is, of course, to be understood that other forms of sensitive elements may be used, and that I do not limit myself to any one form of support or emulsion. All of the operations are carried out at ordinary room temperatures, that is, from 60° to 70° F., except where I have particularly mentioned a temperature used to give a standard result, and in the presence of safe light only, except where otherwise noted. My standard practice, however, is to have all baths at 65° thereby insuring uniformity of working conditions and results.

The theories underlying this process are obscure, and I advance no explanation with confidence. It may be that even after the clearing bath there are left in the sensitive layer small amounts of manganese dioxide or other product of the reversing bath that have a destructive effect on the latent image and these are distributed in that layer proportionally or differentially according to the original silver image. When the second controlled exposure is made this may effect the latent image more strongly at points corresponding to the high lights in the positive since there are more of the destructive salts at these points. Hence the contrast is greater if the second exposure is not too long.

Another possible theory is that the sensitive particles vary in sensitiveness, that the most sensitive are first affected and the less sensitive unaffected. The high lights would thus cause the development of all the most sensitive particles, while in the shadow portions of the image, many of these would be unaffected. The second printing would then consist of the affecting by light of salts differentially sensitive in accordance with the original subject.

I do know, however, that a controlled second exposure after a standardized clearing bath enables me to control the second print-

ing in a manner comparable to the printing of an ordinary positive from an ordinary negative.

The theory of the action of the alkaline bath in preventing a second reversal in the redeveloping bath is also obscure and I advance no theory as to its action.

A field of usefulness for which this process is peculiarly adapted is the making of motion pictures by amateurs for home use. The great deterrent hitherto has been the expense incidental to the purchase of both positive and negative films. Since the process I have outlined would probably and preferably be performed by a finisher under standardized working conditions, it makes it possible for the amateur to purchase the film, and expose it with the same order of care now necessary for satisfactory results with a hand camera, and have the film treated and reversed by a finisher, without the expense of paying for a second film. For home use the film and picture area may be much smaller than standard commercial film and a camera and projector of simpler design and smaller than the commercial ones may also be used, thus bringing the whole field to a point where the original outlay and the running expense will be comparable with that incidental to the use of a hand camera of good quality.

The process above outlined may be used for the making of a positive from a positive, a sensitive element being exposed either by contact or projection to light from or through the transparency or positive image to be copied, and the steps herein described for making an original positive followed.

Having thus described my invention, what I claim as new and desire to secure by Letters Patent is:

1. In a process of making photographic images by reversal from a photographic light sensitive element, containing an image, the steps of submitting the element to a printing light controlled in accordance with the printing value of the element, and then developing an image in said element.

2. In a process of making photographic positive images by reversal from photographic negative images in a light sensitive element, which process comprises the rendering of the negative image inert and differentially transparent and then developing the sensitive element, the step after such rendering and prior to developing of submitting the element to a printing light controlled in accordance with the printing value of the element.

3. In a process of making photographic images by reversal from photographic images in a light sensitive element, the steps of measuring the printing and developing characteristics of the element and then submitting the element to printing and de-

veloping operations in accordance with the characteristics ascertained.

4. The process of making photographic positive images by reversal from photographic negative silver images in an emulsion containing light sensitive salts and comprising the following steps: the removal of the silver from the emulsion; determining the printing and developing characteristics of the emulsion; submitting it to printing and developing operations controlled in accordance with such ascertained characteristics and removing the undeveloped salts.

5. In a process of making photographic positive images by reversal from photographic negative silver images in a light sensitive element, which process comprises the removal of the silver from the element and the development of the element, the steps after such removal and prior to such development of measuring the printing value of the element and submitting it to a printing light controlled in accordance with the printing value.

6. In a process of making images by reversal from photographic images in a strip of sensitized film, the steps of submitting a series of test portions only of such film to a series of standard printing lights and treating such test portions to ascertain the printing characteristics of the film, submitting the film to a printing light controlled in accordance with the characteristics thus ascertained, and then developing the film.

7. In a process of making positive images in a strip of motion picture film having a sensitive emulsion, in which are inert and transparent photographic images, the steps of submitting test portions only of such film to a standard printing light behind a series of graded density tablets, treating such test portions to ascertain the printing characteristics of the film, submitting the film to a printing light controlled in accordance with the characteristics thus ascertained and developing the film.

8. In a process of making positive images in a strip of motion picture film having a gelatine emulsion containing light sensitive salts and in which are inert and transparent photographic images, the steps of submitting test portions only of such film to a standard printing light behind a series of graded density tablets, developing such test portions to ascertain the printing and developing characteristics of said film, submitting the film to a printing light controlled in accordance with the characteristics thus ascertained, developing the exposed sensitive salts in accordance with the ascertained characteristics and removing the undeveloped sensitive salts.

9. In a process of making photographic images by reversal from photographic

70

75

80

85

90

95

100

100

105

110

115

120

120

125

130

- images in a light sensitive element, which process comprises redevelopment of the sensitive element, the step of submitting the element to an alkaline bath prior to redevelopment. 10. In a process of making photographic positives by reversal from an emulsion containing light sensitive salts and a negative image, which process comprises the removal of the negative image and the development of the light sensitive salts, the steps of submitting the emulsion after the removal and prior to the development to an alkaline bath. 11. In a process of making photographic images by reversal from a gelatine emulsion containing light sensitive salts and a silver image, which process comprises the removal of the silver image, the exposure of the emulsion to light and the development of the sensitive salts, the step of submitting the emulsion to an alkaline bath after the removal and prior to development. 12. In a process of making photographic positives by reversal from a gelatine emulsion containing light sensitive salts and a silver image, which process comprises the removal of the silver image in an oxidizing bath, the clearing of the emulsion by the removal of the products of oxidation, and the redevelopment of the light sensitive salts, the step after clearing and before redeveloping of submitting the emulsion to an alkaline bath. 13. In a process of making photographic images by reversal from an emulsion containing light sensitive salts and a photographic image, which process comprises the removal of the image in a bath leaving objectionable products, the removal of such objectionable products, the exposure to light of the emulsion, and its redevelopment, the step of submitting the emulsion to an alkaline bath after the removal of the objectionable products and prior to development. 14. The method of treating a light sensitive element in which there has been formed an inert transparent image which consists in submitting the element to an alkaline bath, and to a developing bath. 15. The method of treating a light sensitive emulsion in which there is an inert transparent image which consists in submitting the emulsion to an alkaline bath, exposing it to light, and then submitting it to a developing bath. 16. The method of treating a gelatine emulsion containing light sensitive salts and an inert transparent, photographic image which consists in submitting the emulsion to an alkaline bath, exposing it to a controlled printing light in accordance with its printing characteristics, and then submitting it to a developing bath. 17. The method of treating a gelatine emulsion containing light sensitive silver salts and an inert, transparent photographic image which consists in submitting the emulsion to an alkaline bath, ascertaining its printing characteristics, exposing it to a printing light controlled in accordance with the printing characteristics, developing the sensitive salts thus exposed, and removing the undeveloped sensitive salts. 18. The method of treating an element containing light sensitive salts and an inert, transparent photographic image which consists in submitting the element to an alkaline bath, ascertaining its printing and developing characteristics, exposing it to a printing light controlled in accordance with the characteristics, developing the exposed sensitive salts in accordance with the characteristics, and removing the undeveloped salts. 19. A photographic reversal process consisting of the following steps: the formation in a light sensitive element of a silver photographic image; dissolving out the silver image in an oxidizing bath; clearing the products of oxidation from the sensitive element; submitting the element to an alkaline bath; measuring the printing characteristics of the element; exposing the element to a controlled printing light in accordance with such characteristics and developing an image in such element. 20. The method of making a photographic positive image consisting of the following steps: exposing to the controlled action of light a gelatine emulsion containing a light sensitive salt; developing a silver image to a high degree of contrast in the emulsion; dissolving out the silver image by an oxidizing bath; clearing the products of oxidation from the sensitive emulsion; submitting the emulsion to an alkaline bath; measuring the printing characteristics of the emulsion; submitting the emulsion to a controlled printing light in accordance with such characteristics; developing the salts affected by the light also in accordance with such characteristics; and removing any undeveloped salts still in the element. 21. The method of treating a light sensitive element in which there is an inert transparent image which consists in testing such element to determine its characteristics as to re-reversal, submitting it to an alkaline bath if it shows a tendency toward re-reversal and then to a developing bath. 22. In a process for making photographic images by reversal from photographic images in a light sensitive element, the step of testing the element to determine its characteristics as to its tendency toward re-reversal and as to its printing value and submitting it to suitable chemical treatment to overcome a tendency to reversal, if any, 120 125 130

and to a controlled printing light in accordance with the results of such steps.

23. In a process for making photographic images by reversal from photographic images in a light sensitive element, the step of testing the element to determine its printing value and its tendency toward reversal, submitting it to an alkaline bath, if it shows a tendency toward re-reversal, 10 submitting it to a printing light controlled in accordance with the printing value and developing said element.

24. In a process for making photographic images by reversal from photographic images in a light sensitive element, the step 15 of testing the element to determine its characteristics regarding re-reversal and development, submitting it to an alkaline bath if it shows a tendency toward re-reversal 20 and developing it in accordance with the results of such test.

25. In a process for making photographic images by reversal from photographic images in a light sensitive element, the step 25 of testing the element to determine its characteristics relating to its tendency toward re-reversal, printing value and contrast, and subjecting it to suitable chemical treatment to overcome a tendency to reversal, if any, 30 controlled printing and controlled develop-

ment in accordance with the results of such steps.

26. In a process for making photographic images by reversal from photographic images in a light sensitive emulsion, the step 35 of testing the emulsion to determine its characteristics relating to its tendency toward re-reversal, printing value and contrast, submitting it to an alkaline bath if it shows a tendency toward re-reversal, and 40 to controlled printing light and development in accordance with the results of such steps.

27. In a process for making photographic images by reversal from a gelatine emulsion containing light sensitive salts and a silver photographic image, the steps of removing the silver image, submitting the emulsion to a clearing bath, testing the emulsion to ascertain its characteristics as 50 to its tendency toward re-reversal, printing value and contrast, submitting it to an alkaline bath if it shows a tendency toward re-reversal, submitting it to a printing light controlled in accordance with the printing 55 value, developing the light affected salts, and removing the undeveloped salts.

Signed at Rochester, New York, this 24th day of February, 1921.

JOHN G. CAPSTAFF.

**Certificate of Correction.**

It is hereby certified that in Letters Patent No. 1,460,703, granted July 3, 1923, upon the application of John G. Capstaff, of Rochester, New York, for an improvement in "Photographic Reversal Processes," errors appear in the printed specification requiring correction as follows: Page 4, line 7, for the word "from" read *front*; same page, line 40, strike out the word "that", and line 53 for the word "proportion" read *proportions*; and that the said Letters Patent should be read with these corrections therein that the same may conform to the record of the case in the Patent Office.

Signed and sealed this 31st day of July, A. D., 1923.

[SEAL.]

KARL FENNING,  
*Acting Commissioner of Patents.*